

# UNITED STATES PATENT OFFICE.

CHARLES A. ERNST, OF LANSDOWNE, PENNSYLVANIA, ASSIGNOR TO SILAS W. PETTIT, OF PHILADELPHIA, PENNSYLVANIA.

## FORMING FILAMENTS OUT OF VISCOSE OR SIMILAR VISCOUS MATERIAL.

No. 863,793.

Specification of Letters Patent.

Patented Aug. 20, 1907.

Application filed April 27, 1907. Serial No. 370,537.

To all whom it may concern:

Be it known that I, CHARLES A. ERNST, a citizen of the United States, and a resident of Lansdowne, State of Pennsylvania, have invented certain new and useful Improvements in Forming Filaments Out of Viscose or Similar Viscous Material, of which the following is a full, clear, and exact description.

My invention relates to the method of forming filaments of cellulose from viscose or similar viscous material and more particularly to the production of the viscose itself, the objects of my invention being to shorten the time of storage heretofore required for the production of viscose, suitable for the formation of filaments, and to preserve the same, to produce a viscose which is speedily coagulated when ejected from the spinneret into the fixing bath, and to increase the strength and elasticity of the filament finally formed.

In making filaments out of viscose, or similar viscous substances, a cellulose base, which may be wood pulp, cotton or any other suitable form of cellulose, is subjected to the action of a solution of caustic soda for a suitable length of time (1 to 4 days) as a result of which the pulp or cotton is changed into soda-cellulose. This product, soda-cellulose, is then placed in a xanthizing machine, comprising a closed receptacle, provided with any suitable means for thoroughly agitating the contents thereof, and a suitable quantity of carbon bi-sulfid is added. The xanthizing machine is then set in motion and the contents thoroughly stirred or agitated, whereupon the soda-cellulose, which is relatively insoluble in water, caustic soda, and similar solutions, is changed into a substance commonly known as cellulose xanthate, which is still solid but which is soluble in the said solutions. To the cellulose xanthate is then added a suitable quantity of one of the above said solvents for the same and a viscous liquid, commonly known as viscose is produced. A filament is then formed from the viscose by ejecting the viscose through minute apertures in a spinneret into a coagulating or neutralizing bath, the function of which is to neutralize the caustic soda in the viscose and to precipitate the xanthate.

Freshly formed viscose would be coagulated and transformed into cellulose by ejecting it through a spinneret into a strong acid bath, but a thread or filament of the same could not be formed commercially, because the cellulose resulting from such treatment or process is very weak and possesses little or no elasticity. To spin a strong elastic thread the viscose must be ejected into a weak neutralizing bath, or in other words it is necessary to employ or produce a viscose which will coagulate immediately into a filament when it is ejected into a weak neutralizing bath. Heretofore, in order to produce a viscose from which

filaments can be spun commercially, it has been necessary to allow the freshly formed viscose to stand or "age" in storage receptacles. It is well known, however, by those skilled in the art, that if the viscose formed in the manner above described, (that is to say by dissolving the cellulose xanthate in a suitable solvent) be allowed to stand or "age" for a sufficient length of time it will of itself change or coagulate, it will be apparent that the function of the "aging" process is to allow the viscose to approach but not quite reach that critical point at which it of itself coagulates, so that all that is needed to transform it into a filament is to spin it into a weak neutralizing bath. But on account of the fact that it is impossible to obtain absolutely uniform cellulose xanthate by the xanthizing process, the result is that during the "aging" process certain portions or parts of the viscose will "age" too much, and particles will frequently coagulate and change into dark colored compounds, which greatly interfere with the spinning by clogging the minute apertures in the spinneret and therefore materially depreciate the quality of the threads or filaments produced. This coagulating of parts of the viscose appears to be due to the further action of carbon bi-sulfid upon the cellulose during the aging process. Moreover during the time required for the "aging", the discoloring impurities in the viscose constantly increase, on account of the formation of sodium-sulfo-carbonates and sulfids.

The object of my invention is, first to produce a viscose which does not require to be "aged" but will coagulate immediately upon its injection into a weak acid bath, although the viscose be fresh, and to preserve the viscose, and second to so check the action of the carbon bi-sulfid as to enable me to store the same until it is needed for spinning, without producing any of the undesirable results above set forth. I accomplish the first of these results by dissolving a suitable quantity of a neutral salt in the solvent for the cellulose xanthate, before the cellulose xanthate is added thereto. In other words I dissolve cellulose xanthate in a solution of caustic soda or of any other suitable solvent containing a soluble salt. I have found that the salts of sodium are particularly adapted to my purpose and I may use sodium-carbonate, sodium-sulfite, sodium-silicate or any other similar salts, since they impart to the viscose the property of coagulating immediately when ejected into a weak neutralizing bath.

The second object, namely, that of checking the further action of the carbon bi-sulfid upon the cellulose and to combine with those impurities in the viscose, which would otherwise discolor the same, is accomplished by adding to the solvent for the cellulose xanthate a suitable quantity of a neutral salt, prefer-

ably a soluble sulfite. In actual practice I find sodium sulfite to be particularly applicable for the purpose.

In carrying out my process I dissolve cellulose xanthate in a weak solution of caustic soda to which has 5 been added a suitable quantity of sodium sulfite and to coagulate the viscose into filaments by spinning them into a neutralizing bath composed of sodium bi-sulfite, which is sufficiently acid for the purpose of coagulating the viscose and is not so expensive as to make the process 10 commercially impracticable.

Another advantage of using sodium sulfite as the salt which is added to the solvent, is that it introduces into the setting or coagulating bath no new chemical element and makes it comparatively easy to reclaim any of 15 the by-products or agents after they have become exhausted, without any difficult or unusual manipulation or processes, although the addition of any other suitable neutral salt or combination of salts, which will produce the results above set forth, may be substituted therefor 20 as they are fully within the scope and aim of my invention. I do not wish, however, to limit myself to a coagulating or neutralizing bath composed of a solution of sodium bi-sulfite since a solution of ammonium chlorid or ammonium sulfate, or a weak solution of almost any 25 other acid may be employed with satisfactory results.

The action of the weak acid bath upon the viscose is merely to transform the liquid cellulose xanthate into a solid filament of cellulose xanthate; that is to say it merely coagulates the viscose into a thread or filament. 30 In order to complete the transformation of the viscose into cellulose or artificial silk, these filaments after being wound upon spools in any suitable manner, are immersed in a bath of sodium bi-sulfite and allowed to stand for a considerable length of time. After this the 35 threads are washed and dried and spun together in any of the usual and well known methods of spinning filaments.

While I have described one way in which my process of forming filaments out of viscose may be performed, I do not desire to be construed as being limited 40 to such, inasmuch as my invention contemplates the introduction into the viscose of any suitable agent or agents, the action of which is to render fresh viscose suitable for spinning and to prevent the undesirable 45 effects of a continued action of carbon bisulfid upon the cellulose.

Having thus described my invention what I claim and desire to protect by Letters Patent of the United States is:

50 1. The process of forming viscose for the production of cellulose filaments, which consists in treating soda-cellulose with carbon bi-sulfid to form cellulose xanthate and then dissolving the said xanthate in a solution containing a substance which will prevent the further action 55 of the carbon bi-sulfid on the cellulose.

2. The process of forming viscose for the production of cellulose filaments which consists in treating soda-cellulose with carbon bi-sulfid and forming cellulose xanthate and then dissolving the said xanthate in a solution con-

taining a substance which will cause the said viscose to 60 coagulate under the action of a weak neutralizing solution.

3. The process of forming viscose for the production of cellulose filaments, which consists in dissolving cellulose xanthate in a solution containing a substance which will 65 cause the viscose, so formed, to coagulate rapidly under the action of a weak neutralizing solution.

4. The process of forming viscose for the production of filaments which consists in adding to a solvent for cellulose xanthate, a salt which will cause the immediate 70 coagulation of the resulting viscose upon its contact with a weak neutralizing solution.

5. The process of forming a filament which consists in forming cellulose xanthate and dissolving the same in an alkaline solvent to which has been added a neutral salt, 75 and then ejecting the resulting viscose into a weak neutralizing bath through minute apertures.

6. The process of forming a filament of cellulose which consists in changing cellulose to soda-cellulose, changing soda-cellulose to cellulose xanthate, dissolving the cellulose xanthate in an alkaline solvent containing sodium sulfite and then coagulating the viscose so formed by ejecting it into a weak acid bath. 80

7. The process of forming a filament which consists in ejecting freshly formed viscose containing a sulfite into 85 a coagulating bath having a slightly acid reaction.

8. The process of forming a filament of cellulose, which consists in ejecting freshly formed viscose containing sodium-sulfite into a coagulating bath having a slightly 90 acid reaction.

9. The process of forming a filament of cellulose which consists in changing cellulose to soda-cellulose, changing soda-cellulose to cellulose xanthate, dissolving the said xanthate in a solution containing a sulfite and then coagulating the viscose so formed by ejecting it into a 95 weak neutralizing bath.

10. The process of forming a filament of cellulose which consists in changing cellulose to soda-cellulose, changing the soda-cellulose to cellulose xanthate, dissolving the cellulose xanthate in an alkaline solvent containing 100 sodium-sulfite, then coagulating the viscose so formed by ejecting it into a weak acid bath, and then subjecting the filament to the continued action of a weak acid bath.

11. The process of forming a filament, which consists in subjecting cellulose to the action of caustic soda to 105 produce soda-cellulose, then adding carbon bi-sulfid to the soda-cellulose to form cellulose xanthate, and then dissolving the said cellulose xanthate in a solution composed of a solvent for the xanthate and sodium-sulfite.

12. The process of forming a filament of cellulose which 110 consists in dissolving cellulose xanthate in an alkaline solvent containing sodium-sulfite, then coagulating the viscose so formed by ejecting it into a bath composed of the solution of sodium bi-sulfite and then subjecting the filament to the continued action of a weak solution of 115 sodium bi-sulfite.

13. The process of forming a filament of cellulose which consists in dissolving cellulose xanthate in a weak solution of caustic soda to which has been added sodium sulfite, ejecting the viscose so formed into a weak sodium 120 bi-sulfite bath, and immersing the filaments in another weak sodium bi-sulfite bath for a sufficient length of time to completely change the coagulated viscose into cellulose.

In witness whereof, I have hereunto set my hand this 125 26th day of April, 1907.

CHARLES A. ERNST.

Witnesses:

ALSTON B. MOULTON,  
ALEXANDER PARK.